

## UNITED STATES PATENT OFFICE

2,220,123

## COLOR PHOTOGRAPHIC PROCESS

László Schwarz, Brussels-Uccle, Belgium, assignor to Béla Gáspár, Hollywood, Calif.

No Drawing. Application September 30, 1939, Serial No. 297,407. In Great Britain October 1, 1938

4 Claims. (Cl. 95—6)

The present invention relates to a color photographic process in which dye images are produced by color development in a layer which contains a color coupler which couples with the 5 oxidation products of the developer to form a dye image.

According to the present invention the color coupler necessary for carrying out this process is produced during the treatment of the exposed 10 silver halide emulsion layer by the destruction of a dye which during the exposure of the light-sensitive layer has the function of a filter dye.

The principal elements of the invention are:

- 15 (a) The presence, in at least one of the silver halide emulsion layers of a light-sensitive multilayer material, of a filter dye, i. e. of a dye which transmits certain colored light rays, required for the exposure of the silver halide emulsion layer or for the exposure of the silver halide emulsion layers, if any, which have to be exposed through said layer, but absorbing other light rays which are not to be recorded by said layer or layers.
  - 20 (b) The filter dye is non-removable by washing and is, if necessary, fixed to the layer by a precipitant.
  - 25 (c) The filter dye is destroyable by chemical means and if thus destroyed yields a compound which is capable of forming a dye by the process of colored development.
  - 30 (d) Destruction of the filter dye is carried out simultaneously with or prior to subjecting the latent image or a residual silver halide image or a bleached out silver image to a developer the oxidation products of which couple with the color coupler to form a dye image.
  - 35 The invention has the advantage that instead of both a filter dye and a color coupler, one substance only has to be incorporated into the light-sensitive emulsion. Mutual interaction of substances of different kind becomes impossible.
  - 40 Furthermore, dyes can be fixed to an emulsion layer in a more efficient manner than can color formers. Dyes from which color couplers are obtained by destruction of the dye are superior to dyes which per se are color couplers, as they do not couple to form a dye as long as they are not destroyed. For this reason it is unnecessary, after the formation of the dye image to remove the color former from the areas where it has not been transformed into dye.
  - 45 The invention consists in the process of pro-
- ducing multicolor dye images by color development in which the filter dye present in at least one of the light-sensitive silver halide emulsion layers of a multilayer material is capable of being destroyed and transformed into a color 5 coupler, and in which the light-sensitive material is exposed and after the first or second development or after transforming the silver image into silver halide, the filter dye is destroyed simultaneously with or prior to the color development 10 of silver halide.
- Dyes from various groups of dyes, such as azo dyes and dyes of the general formula
- (  $\begin{array}{c} \text{C}=\text{O} \\ | \\ \text{CH}-(\text{CH}=\text{CH})_n-\text{CH}=\text{C} \end{array}$  ) 15 )
- described in the co-pending application Ser. No. 240,860 filed November 16, 1938, by Béla Gaspar, are suitable for carrying out the process. Various methods may be used for converting the dye into 20 the color coupler.
- Example.*—A double coated film and a single coated film are united to form a bipack. The single coated film carries an ordinary blue-sensitive silver halide emulsion layer. The double coated film carries on the same side of the transparent support an orthochromatic emulsion in superposition to a panchromatic emulsion layer. Both films are placed together with the three light-sensitive emulsion layers between the supports, the single coated film being the front element of the bipack. Of the two layers of the double coated rear element of the pack the orthochromatic layer is dyed yellow with 0.5 gram 25 per sq. m. of the yellow monoazo dye obtainable by coupling in soda-alkaline solution 1 mol diazotized sulfanilic acid with 1 mol 1.1'-[diphenylene-(4.4)]-bis-[3-methyl-pyrazolone-(5)] (see Beilstein, IVth ed., Suppl. Vol. XXIV, page 212). The panchromatic layer is dyed with 0.3 gram per 30 sq. m. of the redviolet monoazo dye which is obtained by coupling in alkaline solution 1 mol of diazotized sulfanilic acid with 1 mol 1.5-di-hydroxynaphthalene (see Beilstein, IVth ed., Vol. VI, page 980). The bipack is exposed in the camera 35 with the support of the single coated film turned towards the lens. The two elements of the exposed bipack are separated and developed with an ordinary black and white developer and then fixed with hypo. The double coated film is treated 40 thereafter with a solution of 1.5 parts sodium hydrosulfite and 0.1 part anthraquinone- $\beta$ -sulfonic acid in 100 parts of water, rendered slightly alkaline by the addition of sodium carbonate. After the dyes have been more or less decolorized, 45
- 50
- 55

the film is rinsed in water and treated for a few minutes with a 10% aqueous solution of formaldehyde, again washed and treated with an acid cupric chloride solution which transforms the silver images into silver salt images. The film is then subjected to the action of a color developer of the following formula:

|                                          | Parts |
|------------------------------------------|-------|
| 10 p-Dimethylamino-aniline-hydrochloride | 2     |
| 10 Sodium carbonate                      | 30    |
| 10 Water                                 | 1,000 |

The silver images are removed in the known manner, for example with Farmer's reducer and a two-color-negative is obtained in the rear element of the bipack. From the yellow azo dye there has been obtained by reduction with hydro-sulfite a color former which yields a magenta dye by color development and the color former obtained by reduction from the redviolet azo dye is transformed into a bluegreen image. The two-color-image obtained can be printed onto the double coated side and the black-white negative obtained in the front element of the bipack can be printed onto the single coated side of a three-layer-film, having on the one side a blue-sensitive emulsion layer with a coupler for yellow and having on the other side a green-sensitive layer containing a coupler for magenta and a red-sensitive layer containing a coupler for bluegreen. By color developing the positive film, a positive in natural colors is obtained.

Instead of using color couplers in the positive material, there may be used dyes that act as filter dyes and yield the color coupler after destruction. Thus the dyes used in the negative material described above may be employed for coloring the corresponding layers of the positive material. The blue-sensitive layer of the positive film may contain one of the known color couplers for yellow, such as  $\alpha$ -chloro-aceto-acetic ester or a derivative thereof. Alternatively, the blue-sensitive layer may be produced without any color coupler and the yellow dye formed with a color developer of the following formula:

|                                        |       |       |
|----------------------------------------|-------|-------|
| 45 $\alpha$ -Chloro-aceto-acetic ethyl | grams | 2     |
| 50 p-Dimethylamino-amine hydrochloride | grams | 2     |
| 50 Acetone                             | ccs   | 20    |
| 50 Potassium carbonate                 | grams | 40    |
| 50 Water                               | ccs   | 1,000 |

This developer is applied to the single coated side of the positive film, or in the case in which all of the layers of the positive film are on the same side of the support with the blue-sensitive layer on top of the other layers, the action of the color developer is restricted to the top layer and development of the lower layers is continued with a color developer free from color couplers.

60 Whereas in the above example azo dyes have been used the following description shows that also other dyes which are destroyable to form a color coupler may be used for carrying out the process.

65 A light-sensitive silver halide emulsion layer containing 1.5 grams per sq. m. of the yellow dye 4.4'-methylene-bis-[1-(p-sulfophenyl)-3-methyl-pyrazolone-5] is developed with an ordinary black and white developer containing sodium sulfite. The developer destroys the yellow filter dye. After removing the unexposed silver halide

by hypo, the silver image is transformed into a silver halide image by an acid cupric chloride solution and thereafter the film is subjected to a developer containing p-dimethylamino-aniline. The silver is removed by Farmer's reducer and a redviolet dye image is obtained.

Instead of using an ordinary black and white developer, the exposed film may be treated directly with an alkaline p-dimethylamino-aniline developer. This developer acts to destroy the filter dye and to form the dye by the interaction of the color coupler thus obtained with the oxidation products of the developer.

What is claimed is:

1. A process of producing by color development photographic dye images from an exposed light-sensitive silver halide emulsion layer, said light-sensitive silver halide emulsion layer comprising a dye which is destroyable to a color coupler capable of forming a dye by reaction with the oxidation products of a photographic developer, the process comprising treating the layer with a dye destroying agent which acts to transform the dye into said color coupler throughout the layer and with a developer the oxidation products of which form a dye with the coupler at the places where silver halide is transformed to metallic silver. 15

2. A process of producing by color development photographic dye images from an exposed light-sensitive silver halide emulsion layer, said light-sensitive silver halide emulsion layer comprising a dye which is destroyable to a color coupler capable of forming a dye by reaction with the oxidation products of a photographic developer, the process comprising treating the layer with a solution containing both a dye destroying agent which acts to transform the dye into said color coupler throughout the layer and a developer the oxidation products of which form a dye with the coupler at the places where silver halide is transformed to metallic silver. 30

3. A process of producing by color development photographic dye images from an exposed light-sensitive silver halide emulsion layer, said light-sensitive silver halide emulsion layer comprising an azo dye which is destroyable to a color coupler capable of forming a dye by reaction with the oxidation products of a photographic developer, the process comprising treating the layer with a reducing agent which acts to transform the azo dye into said color coupler throughout the layer and with a developer the oxidation products of which form a dye with the coupler at the places where silver halide is transformed to metallic silver. 45

4. A process of producing by color development photographic dye images from an exposed light-sensitive silver halide emulsion layer in a multilayer material, said light-sensitive silver halide emulsion layer comprising a dye which is destroyable to a color coupler capable of forming a dye by reaction with the oxidation products of a photographic developer, the process comprising treating the multilayer material with a dye destroying agent which acts to transform the dye into said color coupler throughout the layer and with a developer the oxidation products of which form a dye with the coupler at the places where silver halide is transformed to metallic silver. 60

CERTIFICATE OF CORRECTION.

Patent No. 2,220,123.

November 5, 1940.

LASZLO SCHWARC.

It is hereby certified that error appears in the printed specification of the above numbered patent requiring correction as follows: Page 1, second column, line 38, for "(4.4)" read --(4.4)--; and that the said Letters Patent should be read with this correction therein that the same may conform to the record of the case in the Patent Office.

Signed and sealed this 14th day of January, A. D. 1941.

(Seal)

Henry Van Arsdale,  
Acting Commissioner of Patents.